

Aug. 18, 1953

W. C. RAMSEY

2,649,441

CONTINUOUS CELLULOSE NITRATION

Filed April 14, 1950



INVENTOR:  
WILLIAM C. RAMSEY

BY *Bruning and Sutherland*  
ATTORNEYS.

## UNITED STATES PATENT OFFICE

2,649,441

## CONTINUOUS CELLULOSE NITRATION

William C. Ramsey, Glendale, Mo., assignor to  
 Olin Industries, Inc., East Alton, Ill., a corpora-  
 tion of Delaware

Application April 14, 1950; Serial No. 155,879

6 Claims. (Cl. 260—220)

1

This invention relates generally to the nitration of cellulose, and particularly to a process of continuously nitrating cellulose in the form of long strips.

It has heretofore been proposed to nitrate continuous strips of cellulosic material by passing the same through a nitrating bath, as represented, for example, by the United States patent to Berl No. 2,384,415.

In the Berl patent mentioned, the strip of cellulosic material is passed through a baffled tank containing the nitrating acid and, in its passage therethrough, is guided over rollers, so that the web of cellulosic material undergoing nitration travels vertically, or nearly so, between the respective upper and lower rollers, which are disposed in alignment with and beyond ends of the respective baffles.

The results achieved with the prior art processes of continuous strip nitration have been disappointing, with particular regard to uniformity, and the apparatus heretofore provided has been particularly difficult to maintain in continuous operation. In view of the very considerable tension which is necessarily imposed upon the strip of cellulose in order to impart the draft required to pass it over the multiplicity of rollers and about the multiplicity of bends, a limitation was imposed upon the tensile strength of the original cellulosic strip; and, if a weak section were encountered therein, so that a rupture occurred in the process of treatment, it was not at all easy to restore operation of the apparatus.

The object of the present invention, generally stated, is to provide process and apparatus for nitrating strips of cellulosic material wherein the nitration is accomplished with uniformity, and wherein the physical strain upon the strip undergoing nitration is minimized.

Other objects will become apparent to those skilled in the art when the following description is read in connection with the accompanying drawing, which is a diagrammatic view of a nitration apparatus constructed in accordance with the present invention.

In accordance with the present invention, generally stated, a strip of cellulosic material to be nitrated is passed through an elongated tube, having a substantial horizontal extent, but somewhat lower at the center than at its ends. The unnitrated strip is fed into the tube at one end, and withdrawn therefrom at the other, so that the strip undergoing nitration is supported at opposite ends of the tube, and is free to assume

2

some sag therebetween, i. e., within the nitrating bath. The nitrating acids are fed into the end of the tube from whence the nitrated strip emerges, and the spent acids are discharged from the end of the tube at which the unnitrated cellulosic strip enters. Accordingly, the first contact of a given increment of unnitrated strip with the nitrating bath is with acid which is of relatively weak nitrating capacity, but as the strip proceeds, the strength of the nitrating acid gradually increases. In the ascending portion of the tube, however, the strength of the acid with which the strip contacts, although higher than that in the descending portion of the tube, is substantially uniform from top to bottom, so that the extent of nitration of the strip may be controlled by regulating the composition of the nitrating acid; it being understood that the degree of nitration of cellulose is ordinarily dependent upon the strength of the acid last contacted by the cellulose, provided the contact is of sufficient duration.

By permitting the suspended strip of cellulosic material, while undergoing nitration, to sag, the nitrating acid is worked into and through the web, and the nitration expedited. This action may be accentuated by the provision of a roller on the upper side of the web undergoing treatment at the valley of the sag, as thereby the transverse sag is at that position flattened. Accordingly, in its travels through the nitrating tube, the strip of cellulose tends to sag in both the ascending and descending portions of the tube, but at the center thereof the sag is flattened, thus, in effect, expanding and contracting the pores of the cellulosic material in each section of the nitrator.

Referring now to the drawings for an illustrative embodiment of the process and apparatus, 40 cellulosic material is provided in the form of a rolled strip 1, mounted for rotation upon a shaft 2. The strip 3, as it emerges from the roll 1, is delivered into a nitrating tube having a descending leg 4 and an ascending leg 5, connected by a junction header 6. In cross-section, the legs 4 and 5 are preferably oval, having their major axes of a dimension but slightly greater than the width of the strip delivered from roll 1, and having their minor axes sufficient only to accommodate the sagging in the strip undergoing treatment without physical contact with the walls of the tube.

In the header 6, a roller 7 is arranged to ride 45 on the upper side of the strip 3. The tension

exerted to draw the strip 3 through the tube about roller 7 thus tends to straighten the reaches of strip between roller 7 and the opposite ends of the tube, and at the same time flattens the lateral bow in the strip.

At the exit end of the nitrating tube, i. e., at the end of leg 5 remote from header 6, a pair of squeeze rolls 8 are provided, one above and one below the strip 3. The squeeze rolls 8 are positively driven from any suitable source of power, and their rate of rotation will determine the lineal velocity of the strip 3 in passing through the nitrating tube. The squeeze rolls 8 are also radially adjusted so as to wring the nitrated strip substantially free of acid.

Fresh nitrating acid is charged into tube 5 at inlet 9, so that the tube is filled to the level indicated at 10, and the spent acid is discharged through outlet 11 adjacent the cellulose intake end of leg 4.

A drain 12 may be provided at the junction header 6 for draining the acid from the tube whenever necessary.

In order to control the temperature of the nitration, the tube, consisting of legs 4 and 5, may be provided with any suitable heating device, such, for example, as an electrical resistance coil, or steam coils 13, 14, 15, and 16. It is preferable to divide the heating coils into separately controllable sections, in order thereby to vary the temperature lengthwise of the legs 4 and 5. Suitable temperature-indicating or automatic temperature-regulating devices may be provided along the length of the tube, as indicated at 17, 18, 19 and 20.

The cellulose material supplied is in the form of paper, made from any suitable pulp, and, depending upon the end use of the nitrated cellulose, may be more or less pure. For the manufacture of smokeless powder, it is most desirable that the paper be as free as possible of substances other than cellulose.

The nitrating acid may be the usual mixture of nitric acid and dehydrator, such as sulphuric, phosphoric, or acetic acids. Depending upon the extent of nitration desired, the content of nitric acid in the nitrating acid mixture may vary from about 75 per cent to about 50 per cent, and the time period within which a given increment of cellulose remains immersed in the nitrating bath may vary from about 30 minutes to about 120 minutes. The temperature maintained within the nitrator may be varied between about 25° C. and about 65° C.

In a typical case, to produce nitrocellulose having a degree of nitration within the gun-cotton range, for example, 13.45 per cent, the fresh nitrating acid may be composed as follows:

|                               | Percent |
|-------------------------------|---------|
| Nitric acid                   | 73.5    |
| Phosphoric acid ( $H_3PO_4$ ) | 25.8    |
| Water                         | 0.7     |

The acid is delivered to the nitrator at a rate such that ten parts of acid pass therethrough while one part of cellulose is passing therethrough. In this instance a given increment of cellulose was within the acid bath for a period of one hour, at a temperature of 60° C. The spent acid had the following composition:

|                 | Percent |
|-----------------|---------|
| Nitric acid     | 63.5    |
| Phosphoric acid | 30.5    |
| Water           | 6.0     |

Stability tests conducted upon the nitrocellulose in the condition in which it emerged from the nitrator, i. e., without any of the usual neutralizing and purifying treatments, was satisfactory, as shown by the German test results, as follows:

|             | Minutes |
|-------------|---------|
| Salmon pink | 45      |
| Red fumes   | 45      |
| Explosion   | 300     |

By reducing the temperature of nitration to an average of 50°, the nitrogen content of nitrocellulose was 13.33 per cent and the spent acid composed as follows:

|                 | Percent |
|-----------------|---------|
| Nitric acid     | 67.7    |
| Phosphoric acid | 29.9    |
| Water           | 2.4     |

With such an arrangement, when the ratio of fresh acid to cellulose is maintained on the order of ten parts of acid to one part of cellulose or higher, the movement of the acid stream downwardly in leg 5 is sufficient to carry along the water molecules released by any nitration which takes place in that leg, as the change in specific gravity of the acid after the nitration reaction is insufficient to overcome the movement of the acid stream in the opposite direction. Accordingly, the composition of the acid which contacts the cellulose in leg 5 remains very nearly at the initial composition, with the highest nitrogen content, however, at the upper surface of the bath in leg 5.

From the foregoing description those skilled in the art should readily understand the operation and advantage of the process and apparatus hereinbefore disclosed and realize that the invention accomplishes its objects. While one embodiment of the apparatus has been shown in the drawings and hereinbefore described, it is to be understood that the invention is not limited to the details of that showing, but that the same may be varied in accordance with the requirements of any given nitration, consistent with the principle that the nitrating tube be relatively long in the horizontal direction, with only sufficient central depression to maintain the tube substantially filled with nitrating acid, and yet permit the entrance and exit of the cellulosic sheet at an angle such that the natural sag of the sheet between points of suspension at the ends of the tube is reasonably approximated. Accordingly, the foregoing disclosure is to be regarded as illustrative and not limiting, save to the extent indicated in the appended claims.

Having thus described the invention, what is claimed and desired to be secured by Letters Patent is:

1. In the art of nitrating cellulose, the process comprising suspending a strip of cellulose at points substantially spaced horizontally so that the strip sags downwardly between the points of suspension and the freely suspended reaches of strip have substantial horizontal extent, and moving the freely suspended reaches through a bath of nitrating acid, said bath being confined about the strip so that the top level of the bath of nitrating acid immediately above the valley of the strip is substantially below the top level of the bath where the strip enters and leaves it.
2. The process of claim 1 wherein the acid is moved in a direction counter current to the movement of the strip.

## 5

3. The process of claim 1 wherein the acid bath consists of nitric acid, phosphoric acid and water.

4. The process of claim 1 wherein each increment of strip is progressively advanced from the first point of suspension through the descending reach and then up the ascending reach to the second point of suspension.

5. The process of claim 4 wherein the  $\text{NO}_3$  content of the acid bath is higher on the ascending reach than on the descending reach.

6. The process of claim 1 wherein the strip is rolled at the valley of the sag within the acid bath.

WILLIAM C. RAMSEY.

15

References Cited in the file of this patent

## UNITED STATES PATENTS

| Number  | Name | Date         |
|---------|------|--------------|
| 214,148 | Hunt | Apr. 8, 1879 |

20

## 6

| Name         | Date          |
|--------------|---------------|
| Mowbray      | Aug. 12, 1890 |
| Cady         | June 4, 1918  |
| Gress et al. | Feb. 23, 1932 |
| Berl         | Sept. 4, 1945 |
| Litkenhous   | Aug. 10, 1948 |

## FOREIGN PATENTS

| Country       | Date          |
|---------------|---------------|
| Great Britain | 1894          |
| Great Britain | 1899          |
| Germany       | Aug. 19, 1920 |
| France        | June 7, 1924  |